

Dec. 6, 1932.

A. P. HINSKY  
INSULATED ELECTRIC CONDUCTOR AND THE METHOD  
OF APPLYING COLORED SURFACES THERETO  
Filed March 17, 1932

1,890,291



INVENTOR.  
ANTHONY P. HINSKY

BY  
*Donald E. Thompson*  
ATTORNEY

## UNITED STATES PATENT OFFICE

ANTHONY P. HINSKY, OF BROOKLYN, NEW YORK, ASSIGNOR TO E. T. TROTTER & CO.,  
OF BROOKLYN, NEW YORK, A CORPORATION OF NEW YORK

INSULATED ELECTRIC CONDUCTOR AND THE METHOD OF APPLYING COLORED  
SURFACES THERETO

Application filed March 17, 1932. Serial No. 599,431.

This invention relates to insulated circuit wires as well as to a method of producing wires of this class, the fibrous jacket of which is treated with a waterproof and flame retardant compound or compounds as well as with a colored coating in the form of a powdered mineral and a final coating of transparent or colored material to give to the finished product a predetermined color value to distinguish it from other conductors; the invention further relates to the use of the method herein defined in the treatment of other fibrous bodies of any kind or class; and the object of the invention is to provide a conductor of the class specified wherein the powdered mineral of predetermined color value is applied to the fibrous jacket immediately after applying the waterproofing or fire repellent compound thereto or while said compound is still in a warm, tacky state so that the powdered mineral will adhere to the conductor and form a coating thereon, permitting the application of a final coating or film which will operate to support and protect the colored mineral on the conductor; a further object being to provide a method of producing colored conductors of the class specified, wherein the fibrous jacket of the conductor is first treated with two compounds, one of greater viscosity than the other; a further object being to provide a method of producing conductors of the class specified, wherein the separate compounds, minerals or coatings are applied in a successive series of operations, thereby saving unnecessary handling of the product in the process of manufacture and also increasing the volume production thereof; and with these and other objects in view, the invention consists in a conductor of the class and for the purpose specified, constructed in accordance with the method more fully hereinafter described and claimed.

The invention is fully disclosed in the following specification, of which the accompanying drawing forms a part, in which the separate parts of my improvement are designated by suitable reference characters in each of the views, and in which:

Fig. 1 is a diagrammatic view illustrating

the several steps in the method of producing a conductor according to my invention; and,

Fig. 2 is a diagrammatic view of a part of a conductor indicating the application of the separate insulating, waterproof and fire-proof, and coloring materials and compounds thereto.

For the purpose of illustrating one manner of producing conductors in accordance with my invention, I have diagrammatically illustrated in Fig. 1 the several steps in the method and the apparatus employed for this purpose. At this time, it will be understood that I am not restricted to the specific type or arrangement of apparatus nor to the specific steps herein disclosed.

In the drawing, 5 represents a reel of an insulated conductor strand consisting of a wire 6, a body of rubber 7 and a fabric jacket 8 as seen in Fig. 2 of the drawing. The jacket 8 is preferably in the form of a cotton braid, but may be of any desired texture and structure. The insulated wire 5a from the reel 5 first passes into and through a tank 9 containing a waterproofing composition or saturant 10, the latter being heated by a suitable heater 11, positioned below the tank 9, and the wire passes over a guide roller 12 downwardly into the tank and around two sheaves 13 and 14 and then over another guide roller 15 at the opposite end of the tank. In passing through the tank 9, the compound 10 is applied to the jacket 8 as indicated in Fig. 2, and this compound thoroughly impregnates the fibres of the jacket as will be apparent.

From the tank 9, the treated wire 5a passes into and through a tank 16 containing another compound 17 preferably of greater viscosity than the compound 10, and also preferably having fire repellent characteristics. The compound 17 is maintained in a heated state by a suitable heater 18. In passing into and through the tank 16, the wire first passes over a guide roller 19 downwardly around two sheaves 20 and 21, and then over another guide roller 22.

From the tank 16, the wire thus treated passes directly into a hopper or container 23 in which is disposed a powdered colored min-

eral 24, which adheres to the compound 17 by reason of the fact that the latter is still in a slightly heated or plastic or tacky state, but not sufficiently so to in any material way obliterate the color value of the powdered mineral. In passing through the hopper 23, the wire travels around a sheave 25 and then through a die or other device 26 for removing the surplus powder. From the die, the wire passes around a guide roller or pulley 27, and then into and through another tank 28 containing a solution 29, which forms the final coating of the conductor, and which may consist of a transparent material or a colored material of a color consistent with that of the mineral 24. In the use of some types of coating materials, a heater 30 will be employed for maintaining the same in a fluid state, it being understood, however, that the coating material 29 may constitute a colored or colorless varnish, lacquer or the like, in which instance, the use of the heater is not necessary. At this time, it will also be understood that the final coating may be applied by spraying, and at the same time, the excess powdered mineral may be removed from the wire or conductor by agitation rather than by use of the die 26.

After passing through the tank 28, the treated conductor passes through a die 31 which applies the coating 29 to the conductor in a smooth, even and polished state to produce a neat and finished appearance. When the final coating is thoroughly dry, the conductor is coiled upon a receiving reel 32.

In Fig. 1 of the drawing, I have indicated at  $\alpha$  and  $\alpha^2$ , two gaps in the wire or conductor, the gap  $\alpha$  being disposed between the tanks 9 and 17 and the gap  $\alpha^2$  between the die 31 and reel 32. It will be understood that between these points, the wires may be passed through dryers or other drying means to facilitate the setting of the compounds or coatings to the wire, as will be apparent. However, it will be understood that the gap at  $\alpha$  is not absolutely necessary, nor in fact, is the gap  $\alpha^2$  required.

It will also be apparent that my invention is not limited to the application of two distinct coatings or compounds to the fibrous jacket 8 prior to applying the powdered mineral thereto, as a single compound may be employed, upon which the powdered mineral is directly applied. The powdered mineral may consist of a compound of suitable substances containing a color pigment of the desired color, which after compounding and drying into a hard or solidified state, is broken up and ground into powdered or granular form to facilitate its application to the conductor in the manner herein set out.

This powdered substance may be produced from paraffin, carnauba wax, synthetic wax and a small percentum of synthetic resin compounded with each other and with the

color pigment in the manner stated. In using a powdered substance of these ingredients, a certain percentage thereof may be combined with the waterproof and fire resisting compound or be reduced to plastic form thereby, without distorting the outer exposed surface of the powdered substance or mineral or the color value thereof. It will also be understood, however, that other ingredients may be employed in the powdered substance or in producing the same which will in no way become effected by the waterproof and fire resisting compound, but will merely adhere thereto because of the sticky or tacky characteristics of the compound.

With my improved process, the inexpensive black and waterproof, fire repellent compounds may be employed in the treatment of the fabric jacket, without danger of distortion in the color value of the powdered mineral, and this result is accomplished by using the powdered colored mineral rather than a colored solution, in which latter instance, the black compound would tend to change or modify the true color value of the resulting conductor.

It will also be apparent that while I have referred to the application of a powdered mineral to a compound while the compound is in a heated or tacky state, that the compound may be applied and allowed to dry and cool or if it is of a consistency that will not produce a tacky or sticky outer surface, a powdered mineral may be employed which can be heated sufficiently to cause adhesion to the compound when applied thereto. It will be understood that the mineral in this case, will be of such characteristics as to withstand the heat without distortion of the color value thereof. However, in some instances, the mineral may be heated to a slight extent, sufficient to cause adhesion thereof to the compound. It will be further understood that the compound need not necessarily be heated in its application to the insulation of the conductor, as the compound may be dissolved in a solvent and applied cold.

It will be understood that my invention is not limited to the production of a cable in accordance with the specific elements herein defined nor in accordance with the process or method set out, and various other changes in and modifications of the structure and method herein defined may be made within the scope of the appended claims without departing from the spirit of the invention or sacrificing its advantages.

Having fully described my invention, what I claim as new and desire to secure by Letters Patent is:

1. The process of treating the insulated jacket of an electric conductor which comprises first applying a liquid compound to the jacket, then applying to the jacket a pow-

dered colored substance having sticky characteristics when subjected to heat, and then covering the powdered substance with a film, retaining said substance against displacement from the jacket of the conductor.

5 2. The process of treating the insulated jacket of an electric conductor which comprises first applying a liquid compound to the jacket, then applying a powdered colored substance including a binder to the jacket treated with the compound, and then covering the powdered substance with a film, retaining said substance against displacement from the jacket of the conductor, and applying 10 the powdered substance to the jacket while the compound is in a plastic state to insure adhesion between the powdered substance and compound.

15 3. The process of treating the insulated jacket of an electric conductor which comprises first applying a liquid compound to the jacket, then applying a powdered coating comprising a color pigment and a binder to the jacket treated with the compound, and then covering said coating with a film of 20 transparent material forming an outer protector sheath for the powdered coating, through which the color value of the powdered coating is visible.

25 4. A process of treating the fibrous covering of an insulated electric conductor which consists in first applying a black waterproofing saturant to said covering, then applying a black flame repellent compound thereto, 30 then applying a colored powdered mineral including a wax binder to the covering treated with the compounds so as to cause adhesion of the powdered mineral to the conductor, and then enclosing the conductor thus 35 formed in an outer film for supporting the powdered mineral thereon.

40 5. A process of treating the fibrous covering of an insulated electric conductor which consists in first applying a black waterproofing saturant to said covering, then applying a black flame repellent compound thereto, 45 then applying a colored powdered mineral including a wax binder to the covering treated with the compounds so as to cause adhesion 50 of the powdered mineral to the conductor, then enclosing the conductor thus formed in an outer film for supporting the powdered mineral thereon, and employing in the film coating a material of a color value 55 consistent with that of the powdered mineral.

60 6. A process of treating the fibrous covering of an insulated electric conductor which consists in first applying a black waterproofing saturant to said covering, then applying a black flame repellent compound thereto, 65 then applying a colored powdered mineral including a binder to the covering treated with the compounds so as to cause adhesion of the powdered mineral to the conductor, removing the surplus powdered mineral from

the conductor, and then enclosing the conductor thus formed in an outer film for supporting the powdered mineral thereon.

7. The herein described process of applying an opaque colored jacket to the insulation 70 of an electric conductor, which consists in first treating the insulation with a waterproof and flame repellent compound, then covering the treated insulation with a jacket consisting of colored opaque particles having 75 sticky characteristics when subjected to heat and adhering to said treated insulation, and then enclosing said jacket in a coating maintaining the color value of said jacket.

8. The herein described process of applying an opaque colored jacket to an elongated, fibrous strand, which comprises first treating the strand with a compound having sticky characteristics, then covering the treated strand with a jacket consisting of colored 80 opaque particles including a binder, said particles adhering to and enveloping said compound, and then enclosing said jacket in a coating maintaining the color value of said jacket and giving predetermined color value 85 to said strand.

9. A process of treating a fibrous strand to give predetermined color value thereto, which comprises first treating the strand with a heated fluid, then applying a colored powdered mineral including a binder to the compound on the strand while in a heated state to insure adhesion of the powdered mineral thereto, removing the surplus mineral to form a colored jacket evenly disposed on said strand, and then enclosing the colored jacket with a coating maintaining the powdered substance of the jacket against accidental 95 displacement from the strand.

10. The herein described method of producing elongated fibrous strands of the class described with outer coatings of predetermined color, which consists in first treating the strand with a compound impregnating the fibres thereof, then applying another compound to said strand having a viscosity greater than that of the first compound, then applying a colored powdered substance comprising a color pigment and a wax-like binder 100 to the last compound to cause adhesion between the powdered substance and viscous compound without disturbing the outer color value of the powdered substance, and then applying a retaining coating or film to said powdered substance maintaining the color 105 value of said powdered substance.

11. The process of treating a predetermined surface, which comprises first applying a compound thereto, then applying a powdered coating comprising a colored pigment and a binder having sticky characteristics to the compound, and then covering the powdered coating with a film retaining said coating against displacement from the surface.

12. In the art of applying coatings to a fibrous, strand-like body, a compound having sticky characteristics applied directly on said body, a colored powdered substance including a binder enveloping the compound and adhered thereto by the sticky characteristics of the compound, and an outer coating enveloping the powdered substance and retaining the color value thereof.
- 10 13. In the art of electrical insulation, an electric wire with an insulating jacket, said jacket being treated with a waterproof and fire resistant compound, a colored powdered coating including a binder enveloping the compound and adhered thereto, and an outer coating of transparent material enveloping said coating.
- 15

20 In testimony that I claim the foregoing as my invention I have signed my name this 16th day of March, 1932.

ANTHONY P. HINSKY.

25

30

35

40

45

50

55

60

65